

June 24, 1924

1,498,735

W. T. KRAUSCH  
SMOKEJACK AND THE LIKE

Filed Jan. 2, 1923



16  
Witnesses  
Milton Lenoir  
Bill Morell

15  
10  
16  
15  
12  
15  
16  
10  
15  
16  
15  
12  
15  
16  
15  
16  
17  
18  
19  
20  
Inventor  
Walter T. Krausch,  
George Heidman  
Attorney

## UNITED STATES PATENT OFFICE.

WALTER T. KRAUSCH, OF LA GRANGE, ILLINOIS.

## SMOKEJACK AND THE LIKE.

Application filed January 2, 1923. Serial No. 610,161.

*To all whom it may concern:*

Be it known that I, WALTER T. KRAUSCH, a citizen of the United States, and a resident of La Grange, in the county of Cook 5 and State of Illinois, have invented certain new and useful Improvements in Smokejacks and the like, of which the following is a description, reference being had to the accompanying drawings, which form a part 10 of my specification.

My invention relates more particularly to an improved smoke jack for use in locomotive or engine houses and the like, although the invention is equally adaptable for use as 15 a ventilator or other similar devices.

The invention has for its object the provision of a construction formed primarily of thin sheet metal, provided preferably both interiorly and exteriorly, that is to 20 say on either or both sides of the metal, with a protective coating adapted to resist fire and to protect the metal against the action of sulphuric fumes as well as the elements. With my invention a smoke jack 25 may be made of materially less weight than has heretofore been the case and as a result the weight on the roof-timbers will be greatly lessened; while at the same time the initial cost, as well as the cost of upkeep, 30 is materially reduced.

The objects and advantages of my invention will be readily comprehended from the detailed description of the drawings, wherein:—

35 Figure 1 is an elevation and partial longitudinal section of my improved smoke jack and its mounting on the roof timbers.

Figure 2 is a longitudinal sectional view.

40 Figure 3 is a cross sectional view taken on the line 3—3 of Figure 1 looking in the direction of the arrows.

Figure 4 is a cross sectional view taken on the line 4—4 of Figure 1.

In the particular exemplification of the 45 invention it has been shown in the nature of a smoke jack for an engine house and consists of the conduit or main stack 10 disposed upwardly through a suitable opening in the roof of the building as indicated 50 at 11; the lower end of the stack being provided with a hood or skirt portion 12 flared in the usual manner so as to extend entirely over the smokestack of a locomotive. The lower flared end or skirt portion 12 is suitably supported from the roof timbers or 55 joists indicated at 13 by suitable straps or

hangers 14 which may be bolted to the roof timbers as shown at 15 and riveted or bolted to the lower or flared end of the skirt portion as shown at 16. In order that the skirt 60 portion may have proper flare, it is usual to construct the same of a number of sheets which are riveted together as shown at 17 in Figure 1.

The upper end or stack portion 10 is preferably further supported in vertical position by means of a hood or collar 18 secured about the opening in the roof 11 and the hood portion 18 also preferably constructed of a protected sheet metal similar to that 70 of the jack and as hereinafter described.

My improved jack, throughout, consists of comparatively thin sheet metal which is preferably provided on either or both sides or surfaces with a coating of asbestos material or asbestos sheet; the asbestos (whether in sheet or fibre form) being cemented to the metal with a suitable adhesive material, preferably by means of liquid glass or front end cement. After the cementing 80 material, which is applied throughout the entire surface of the stack, has become thoroughly "set" so as to securely cement the asbestos to the metal, the entire asbestos 85 surface, namely the asbestos coating on the interior and exterior of the stack or on both sides or surfaces on the sheet metal, is then given a coating consisting preferably of liquid glass sufficient to thoroughly fill the pores or interstices of the asbestos covering or layer.

In employing the invention as disclosed in the drawing, the sheet metal is first cut and formed into shape to provide a smoke jack or ventilating conduit of the desired configuration or shape and preferably with a lap joint as shown at 19 in Figure 4; the lapped metal being preferably suitably riveted as at 20. The smoke jack or ventilating conduit of sheet metal, on both the 100 inner and outer surfaces thereof, as well as the lapped and riveted portion thereof, is provided with an adhesive coating, preferably of front end cement or of liquid glass, to which a coating or covering of plastic or 105 sheet asbestos material is then applied before the coating or liquid glass has become set. The adhesive or cementing material, with the asbestos covering, is then allowed to "set" or harden and the outer surface of 110 the asbestos material or protective covering is then preferably provided with a coating

of liquid glass in quantity sufficient to fill the pores or interstices of the asbestos; the outer coating of glass being allowed to dry before the smoke jack is erected or put into use.

With my invention, a smoke jack or ventilating conduit is provided which will resist the action of fire and sulfuric fumes as well as the action of the elements; while at the same time comparatively thin sheet metal may be employed and consequently the weight and cost materially reduced and as a result the weight on the roof-timbers materially decreased.

It is apparent that my improved method and the resultant material may be employed for other purposes or conduits where it is subjected to gaseous fumes or exposed to the elements and that materially thinner sheet metal may be used than has heretofore been the case while at the same time being capable of resisting the destructive action of the elements or fumes for a longer period of time, thereby greatly reducing the cost of maintenance.

What I claim is:

1. A smoke jack composed of sheet metal formed into shape, and an inner and outer covering of asbestos cemented to the metal 30 to constitute a unit therewith.

2. A smoke jack composed of sheet metal cut and riveted into shape, asbestos intimately secured to the metal by a cementitious material, and a coating of gas resisting material for impregnating the asbestos.

3. An article of the character described, composed of sheet metal, a layer of asbestos cemented into intimate relation with the metal, and a coating of liquid glass applied to the outer surface of the asbestos.

4. A smoke jack composed of sheet metal, the inner and outer surfaces of the jack being provided with asbestos cemented thereto to provide a unitary structure, and a coating of liquid glass on the exposed surface of the asbestos.

5. The herein described method, which consists in forming a smoke jack or conduit out of sheet metal, coating the inner and outer surfaces of the smoke jack or conduit with liquid glass, applying asbestos to said coating of liquid glass, allowing the liquid glass to set or dry and then coating the exposed surface of the asbestos with liquid glass.

WALTER T. KRAUSCH.

Witnesses:

FRED C. GARRETT,  
ROBERT H. SALISBURY.